

[54] THIN FILM DIELECTRIC STORAGE TARGET AND METHOD FOR MAKING SAME

[75] Inventor: Wolfgang M. Feist, Burlington, Mass.

[73] Assignee: Raytheon Company, Lexington, Mass.

[22] Filed: Nov. 27, 1973

[21] Appl. No.: 419,302

**Related U.S. Application Data**

[60] Division of Ser. No. 355,855, April 30, 1973, which is a division of Ser. No. 208,494, Dec. 15, 1971, abandoned, which is a division of Ser. No. 210,095, Dec. 20, 1971, abandoned, which is a continuation of Ser. No. 12,566, Feb. 19, 1970, abandoned, and a continuation-in-part of Ser. No. 806,534, March 12, 1969, abandoned.

[52] U.S. Cl. .... 96/38; 96/45; 156/3; 156/8; 156/18; 204/24; 313/395; 427/247; 427/331

[51] Int. Cl.<sup>2</sup> .... H01J 31/48

[58] Field of Search ..... 313/66, 65 T, 65 AB, 313/68, 391, 393, 394, 395, 408; 156/3, 18, 8, 11, 17; 29/25.11, 25.17; 204/32 R, 18 PC, 24; 117/130 E; 96/36, 36.1, 36.2, 38.4, 45, 38; 106/55; 427/12, 77, 247, 331

[56]

**References Cited**

UNITED STATES PATENTS

|           |         |                        |         |
|-----------|---------|------------------------|---------|
| 2,985,548 | 5/1961  | Blickwedel et al. .... | 427/77  |
| 3,249,785 | 5/1966  | Floyd et al. ....      | 313/65  |
| 3,398,317 | 8/1968  | Shoulders ....         | 313/394 |
| 3,469,941 | 9/1969  | Kuhn ....              | 106/55  |
| 3,474,511 | 10/1969 | Ort et al. ....        | 313/65  |
| 3,493,803 | 2/1970  | Koda et al. ....       | 313/393 |
| 3,497,747 | 2/1970  | Einstein ....          | 313/395 |
| 3,535,574 | 10/1970 | Maeda ....             | 313/68  |
| 3,535,575 | 10/1970 | Herman ....            | 313/395 |
| 3,564,321 | 2/1971  | Saldi ....             | 313/65  |
| 3,633,064 | 1/1972  | Herman ....            | 313/394 |

Primary Examiner—William A. Powell

Assistant Examiner—Jerome W. Massie

Attorney, Agent, or Firm—John R. Inge; Joseph D. Pannone; Milton D. Bartlett

[57]

**ABSTRACT**

A membrane type dielectric storage target formed from a thin refractory dielectric film is stretched to form at least a one-sided surface, a first surface portion contacting a conductive wire mesh, a second surface portion having areas coated with conductive material imaging the mesh of the first surface portion. The method contemplates forming the conductive image on the second surface portion by photo-resist, decoration, and breakdown techniques.

7 Claims, 4 Drawing Figures





Fig. 1.

Fig. 2.



Fig. 3.



*Fig. 4.*

## THIN FILM DIELECTRIC STORAGE TARGET AND METHOD FOR MAKING SAME

This is a division of application Ser. No. 208,494 filed Dec. 15, 1971, which is a division of application Ser. No. 355,855 filed Apr. 30, 1973, which is a division of application Ser. No. 210,095 filed Dec. 20, 1971 (now abandoned), which is a continuation of application Ser. No. 12,566 filed Feb. 19, 1970 (now abandoned), which is a continuation in part of Ser. No. 806,534 filed Mar. 12, 1969 (now abandoned).

### BACKGROUND OF THE INVENTION

This invention relates to dielectric storage targets and, more particularly, to membrane type dielectric storage targets and methods for fabricating same. This is a continuation in part of U.S. patent application Ser. No. 806,534, filed Mar. 18, 1969.

Dielectric storage films have been used to coat apertured conductive target electrodes in electron beam storage tubes. Such electrodes may take the form of fine wire mesh grids. There are many wire mesh target electrode structures shown in the prior art. Frequently, these structures exhibit thick film dielectric layers contiguous to the wire mesh, the mesh apertures being plugged with conductive material. The metal plugs are inserted in order to offset the combined capacitance effects of the metal mesh and the thin dielectric film coatings. In this regard, reference may be made to Teal (U.S. Pat. No. 2,630,101) and H. R. Day (U.S. Pat Nos. 3,020,433 and 3,116,191). Such prior art structures, however, do not relieve the mechanical stress exerted by the film on the supporting mesh. Also, the use of metal plugs to correct thick film capacitance distortion increases rather than decreases the mechanical burden carried by the wire mesh.

It is, accordingly, an object of this invention to devise a dielectric storage target electrode in which mechanical stress on a supporting mesh is minimized. Relatedly, it is desired to reduce the leakage of charge as well as the capacitance formed by the dielectric membrane element to the surrounding conducting mesh.

In the prior art, the forming of conductive surfaces on either side of a dielectric has required the use only of those dielectrics through which metal will diffuse at elevated temperatures. Thus, a nickel mesh with a gold coating covered with a zinc sulphide dielectric layer permits the gold from the nickel to diffuse through the dielectric onto the other side. Unfortunately, dielectrics such as zinc sulphide are relatively poor and exhibit undesirably high leakage currents if the operating temperature exceeds room temperature. Dielectric membranes formed from higher quality dielectric materials do not readily permit diffusion of a metal therethrough.

It is, accordingly, another object of this invention to devise a membrane type dielectric storage target and method for making same in which the wire mesh support on one surface of the film is exactly imaged on another portion of the dielectric film and further that the dielectric be of high quality. Relatedly, it is desired that the method for fabrication should not be dependent upon the diffusion of metal through the dielectric portion of the target.

### SUMMARY

The aforementioned objects are satisfied in several preferred embodiments and methods for making same.

The invention contemplates a membrane type dielectric storage target in which a thin refractory dielectric film such as boron nitride, is stretched to form a surface to which a conductive wire mesh contiguously and intimately contacts at least a portion of the surface with a conductive image of the wire mesh contiguously and intimately contacting at least another portion of the surface.

The dielectric film is stretched to form an inside and outside surface. In this embodiment, the conductive wire mesh contiguously and intimately contacts at least a portion of the inner surface. Likewise, the conductive image of the wire mesh contiguously and intimately contacts at least a portion of the outer surface.

15 The method for fabricating the membrane type dielectric storage target comprises the steps of coating the metal mesh with a lacquer layer and depositing a thin refractory dielectric film over the lacquer coated mesh. Subsequently, the lacquer layer is removed, as by

20 applying heat to the film. Significantly, an image of the mesh is formed on another surface of the refractory dielectric film using photo-resist, decoration, and electrical breakdown techniques. Lastly, a conductive metal grid is formed on the image portions of the surface in the case of photolithographic techniques.

### BRIEF DESCRIPTION OF THE DRAWINGS

FIG. 1 is a generalized flow diagram.

FIG. 2 is a flow diagram of the photo-resist method of 30 fabricating the membrane storage target.

FIG. 3 is a flow diagram of the decoration method of fabricating the membrane storage target.

FIG. 4 shows an electron beam storage tube including the thin boron nitride dielectric storage target 35 membrane.

### DESCRIPTION OF THE PREFERRED EMBODIMENTS

As previously discussed in co-pending U.S. patent 40 application Ser. No. 806,534, dielectric storage targets are used in electron memory tubes. The information is written on the targets by an electron beam. Operationally, the electron beam charges different areas of the target to the same or different potentials. The information is then read from the target by the same electron beam or a different electron beam, and at a speed which may be substantially different from the writing or energizing process. In the ensuing paragraphs, attention shall first be directed to a number of different 45 geometric embodiments of the membrane target. This will be followed by a discussion of the fabrication of a planar matrix target according to the invention.

The target for dielectric storage has a variety of embodiments which, for example, may consist of a dielectric layer formed on a conducting substrate, a dielectric layer formed on a mesh in such fashion that is partly 55 fills the apertures of the mesh, and a conducting mesh over whose entire area a dielectric film is laid down. In this latter structure, the mesh apertures are filled with 60 membranes.

It is to be understood that the thin film would have attached along one portion of its surface extent an integral self-supporting metal structure in the form of a conductive wire mesh defining a plurality of apertures.

65 The dielectric film, made preferably from boron nitride, contiguously and intimately contacts the mesh including the apertures. A conductive image of the wire mesh which also contiguously and intimately contacts

another portion of the thin film surface completes the basic membrane type storage target. Of course, the film may be shaped as a conventional flat surface in which the wire mesh contacts the film on one side and the conductive image contacts the film on the other side. The wire mesh and its conductive image may, of course, be oppositely disposed one from the other, or for a portion of their extents spatially overlapping. In the case of the one-sided surface, the mesh and its conductive image would occupy distinct non-overlapping surface portions.

The membrane type storage structure of this invention may be made on thin as 1000 to 3000 Angstroms when fabricated according to the hereinafter to be described methods. It is well to consider the advantages that derive from thin membrane type storage targets. First, the deposition time for forming the dielectric films is kept to a minimum. Second, the stresses exerted by the dielectric film on the supporting mesh are reduced due to a smaller mass of film. Third, the leakage current, as well as the capacitance from a dielectric membrane element to the surrounding conducting mesh, is small. This is because of the thinness of the film and the relatively large spacing between the mesh wires. An added benefit deriving from the small capacitance is that the writing speed of electron beam upon the target may be substantially increased.

In the prior art, dielectric storage screens were fabricated according to the following steps. First, a nickel wire mesh in the order of 750 to 1000 meshes per inch was immersed in a tank filled with nitrocellulose lacquer. After removal from the tank, the excess lacquer was spun off the mesh and the remaining lacquer dried to form a membrane covering the screen. A dielectric film was then deposited over the lacquer membrane. Subsequently, the lacquer was removed by heating the mesh in air. For proper functioning as a storage target, it was mandatory that the conducting grid present only on the substrate side of the dielectric film would have to be duplicated in perfect alignment on the outer surface of the dielectric. It was necessary to coat the nickel mesh with a thin layer of a suitable metal such as gold before forming the lacquer membrane. The dielectric was restricted to only those materials which would permit diffusion of the metal at elevated temperatures as for example zinc sulphide. After the dielectric membrane was formed, the screen was heated for a period of time to a suitable temperature. This elevated temperature resulted in the gold diffusing from the grid wires to the opposite surface of the dielectric.

It must be clearly recognized that materials such as zinc sulphide permitting diffusion are comparatively poor dielectrics. Indeed, storage screens fabricated from zinc sulphide exhibit high dielectric leakage at operating temperatures exceeding 20°C to 30°C. As previously suggested, membranes formed with higher quality dielectric materials do not readily permit diffusions of a metal and consequently cannot be used for dielectric storage target fabrication purposes.

Referring now to FIGS. 1, 2, and 3, there are shown respectively flow diagrams of the process steps for making the thin film membranes according to the invention. With attention now to FIG. 1, there are shown five basic steps in forming a conductive image of the dielectric film on another portion of the same surface as well as diametrically opposite the mesh.

The metal mesh is first coated with a supporting layer such as, for example, nitrocellulose. A thin refractory

dielectric film such as boron nitride is deposited on the lacquer coated mesh. The nitrocellulose lacquer base is removed, for example, by applying heat to the refractory covered mesh. An image of the mesh is made opposite or upon another surface or portion thereof on the dielectric film. Lastly, a conductive metal grid is formed on the image portions of the mesh when a photolithographic process is used.

Referring now to FIG. 2 of the drawing, there are shown the detailed steps of image formation utilizing a photo-resist technique. After the lacquer has been removed, the outer or other surface portion of the dielectric film is coated first with a thin conductive metallic film in the range between 200 Angstroms to 500 Angstroms of, for example, gold. Next, a photo-resist layer is spun over the gold and subjected to proper drying and baking. The photo-resist layer is exposed to suitable light such as ultraviolet with the mesh acting as a mask. The exposed photo-resist is then developed and removed only from aperture areas. Now, the gold film is etched away from the aperture areas. Aurostrip was found to be a suitable etchant because it removes the gold without attacking the mesh metal. Lastly, the remaining photo-resist is chemically removed such as by chemical stripping, heating in air, or exposure to an oxygen plasma.

A variation of this technique is also useful. Thus, after the dielectric membrane is formed, the photo-resist is put on, exposed, and developed. This results in photo-resist covering the areas opposite the apertures in the mesh only. Next, a thin gold film is deposited on the side of the outer face or other surface portion of the dielectric membrane. Lastly, the remaining photo-resist is chemically stripped, a process which also washes off the gold film from the areas opposite the mesh apertures.

Referring now to FIG. 3, there is shown a second technique for producing an image of the conductive mesh on the opposite or other surface portion of the dielectric film. Again, after formation of the dielectric membrane and the removal of the lacquer layer, the mesh is immersed in a plating solution of, for example, copper or gold with a negative potential being applied to the mesh. As a result, the copper or gold plates through any pinholes or fine cracks in the dielectric film. However, this only occurs in areas over the mesh wires. This method presupposes the existence of a sufficient number of pinholes in the thin dielectric film. Such a number may be created artificially as, for example, by using a mesh whose wires have a relatively rough surface or by spraying a fine silica or boron nitride dust over the mesh before deposition of the dielectric.

In practice, a plating bath was set up in which the gravity of the bath was adjusted to 16° Baume, the pH level being 4.5 and the temperature being 560° Rankin. The distance between a 2-inch by 3-inch stainless steel anode and the sample was between 1 to 2 inches. It was desired to plate a 2-inch diameter, 1000 mesh grid coated with a BN membrane between 2000 Angstroms to 3000 Angstroms thickness. This was attained with a current level of between 40 to 50 milliamperes for a period of between 2 to 10 minutes. The potential required to achieve this deposition was in the order of 1 to 5 volts.

Lastly, a breakdown technique may be used. First, the dielectric membrane is formed and the lacquer layer is removed. One side of the screen is protected by

lacquer and the front of the film exposed to an electrolyte or a plasma. The electrolyte or plasma makes it possible to apply a potential across the dielectric film which is sufficiently high to cause the desired breakdown to occur at areas over the grid wires. Removal of the lacquer coating by baking in air completes the process.

Referring now to FIG. 5 of the drawings, there is shown an electron beam storage tube 13. The tube comprises an evacuated glass chamber with an electron gun 12 at one end and target electrode means 14 at the other end. An electron beam is formed in the usual manner by the gun 13. The gun includes a cathode 1, a grid 2, and an anode 3. Radiating the beam along its path in the conventional manner are magnetic focusing coil 14, deflection coil 5, and deceleration means 7.

Target electrode means 14 comprises a first screen 13 and a thin boron nitride membrane coating 11 intimately and contiguously contacting at least a portion of storage screen mesh 10. Signal electrode 9 forms a collector reflector to the beam and storage screen mesh membrane 10. The BN storage film does not require a layer of gold because the cross-over voltage is between 20 60 to 90 volts. In view of the fact that the conductive 25 target electrode serves also as a metal substrate, meshes made out of nickel are useful for mounting the thin BN membrane. Molybdenum and tungsten meshes also exhibit good thermal expansion properties at elevated temperatures, thereby avoiding membrane wrinkling.

In the foregoing disclosure, an improved membrane type dielectric storage target has been shown, being shaped in conventional or topologic forms and further including a method for forming a conductive image of the mesh on an opposite or another surface portion by photo-resist, decoration, and breakdown techniques. It should be understood that this invention is not limited to the precise construction herein described in connection with the illustrative drawings but that other embodiments within the scope of the appended claims are to be considered within the purview of the invention.

What is claimed is:

1. A method for making a target for a storage tube comprising:  
coating a metal mesh with a lacquer layer;  
forming a thin substantially transparent refractory dielectric film on said metal mesh;  
removing said lacquer layer;  
depositing a layer of metal on the opposite side of 50 said film from said mesh, said layer of metal having a thickness in the range of 200A to 500A;  
applying a photo-resist layer on said metal layer;

illuminating said photo-resist layer through said mesh with ultraviolet light;  
removing the illuminated portions of said photo-resist layer to expose portions of said metal layer;  
and  
removing said exposed portions of said metal layer by etching.

2. The combination of claim 1 wherein said dielectric film consists of boron nitride.

3. The method of claim 1 wherein said layer of metal consists of gold.

4. The combination of claim 1 further comprising the step of:

chemically removing the remaining photo-resist layer.

5. A method for fabricating a dielectric storage target comprising the steps of:

coating a non-reactive conductive metal mesh with a lacquer layer;

depositing a thin substantially transparent refractory dielectric film on said lacquer layer;

evaporating the lacquer layer by applying heat to the film covered mesh;

immersing the film covered mesh in a plating solution preferably of copper or gold; and

applying a negative potential to the mesh whereby the plating material exudes through the pre-existing fine cracks and pores in the dielectric film in the area of the mesh wires.

6. A method for making a target for a storage tube comprising:

coating a metal mesh with a lacquer layer;

forming a thin substantially transparent refractory dielectric film on said metal mesh;

removing said lacquer layer;

applying a layer of photo-resist upon said dielectric film;

illuminating portions of said photo-resist layer through said metal mesh;

removing portions of said photo-resist layer illuminated through said metal mesh;

depositing a layer of gold over remaining portions of said photo-resist layer and portions of said dielectric film exposed where portions of said photo-resist layer were removed; and

removing said remaining portions of said photo-resist layer and portions of said gold layer deposited upon said remaining portions of said photo-resist layer.

7. The method of claim 6 wherein said dielectric film consists of boron nitride.

\* \* \* \* \*

UNITED STATES PATENT OFFICE  
CERTIFICATE OF CORRECTION

Patent No. 3,960,562 Dated June 1, 1976

Inventor(s) Wolfgang M. Feist

It is certified that error appears in the above-identified patent and that said Letters Patent are hereby corrected as shown below:

Column 1, line 18, change "Mar. 18, 1969" to -- Mar. 12, 1969 --

Column 1, line 30, change "2,630,101" to -- 2,650,191 --

Column 2, line 9, change "stretche" to -- stretched --

Column 2, line 19, change "subsequenting" to -- subsequently --

Column 2, line 56, change "is" to -- it --

Column 3, line 26, insert -- the -- between of & electron

Column 5, line 13, change "gun 13" to -- gun 12 --

Signed and Sealed this

Fourth Day of January 1977

[SEAL]

Attest:

RUTH C. MASON  
Attesting Officer

C. MARSHALL DANN  
Commissioner of Patents and Trademarks